

## UNITED STATES PATENT OFFICE

2,120,616

## LUBRICATING FLUID

William G. Klitzke, Portland, Oreg.

No Drawing. Application March 30, 1937,  
Serial No. 133,907

2 Claims. (Cl. 87—9)

This invention relates to the class of lubrication, and pertains particularly to an improved lubricating fluid designed primarily for lubricating valves and other sliding parts of musical wind instruments.

The present invention has for its primary object to provide an improved free flowing and nondrying lubricating fluid which may be freely used upon valves and other sliding parts of musical wind instruments, such as cornets, trombones or the like, without danger of damaging the metal of the instrument and without becoming eventually gummy so as to require the cleaning of the parts.

The present invention broadly contemplates the provision of a soap in water solution having added thereto an oil or oils which forms the double function of preventing the drying out and gumming of the soap and providing additional lubricant for the parts to which the fluid is applied.

More specifically the invention comprises a mixture or emulsion of water, kerosene, a soap such as the brand commonly sold under the trade name "Ivory", and oil of citronella. In making up the lubricating fluid the water is first heated, and the soap, in the form of "Ivory" soap chips, is dissolved therein. After a complete solution has been effected, kerosene oil is added and thoroughly mixed in so as to form an emulsion.

This emulsion is then permitted to cool and it then has added oil of citronella which will thin out the previously formed thickened liquid.

As a specific example of the invention, it is preferred that the ingredients be taken in the following proportions:

|                                               |         |     |
|-----------------------------------------------|---------|-----|
| Water                                         | gallons | 1   |
| Kerosene                                      | do      | 2   |
| Oil of citronella                             | ounces  | 3   |
| Soap chips or powder (Ivory soap<br>40 chips) | do      | 1/4 |

While the soap preferred for use in this preparation is that sold under the trade name previously referred to, other pure soaps may be employed, therefore it is to be understood that the invention is not to be limited to the use of "Ivory" soap chips.

It is well known that soaps have a certain degree of lubricating action, but in the present case the use of a soap and water solution alone, while effective for a short period of time, would finally defeat the purpose for which it is used by drying out and hindering the movement of the instrument parts between which it might be placed. For this reason the addition of kerosene and citronella oils serves the double function of preventing the drying out of the soap after the water has evaporated and of adding an additional lubricant to the mixture. The combination of the kerosene with the soap and water mixture also tends to retard the evaporation of the water of the mixture.

What is claimed, is:

1. A lubricating fluid for the purpose described, comprising an emulsion consisting of a mixture of a fully formed soap, water in which the soap is dissolved, kerosene oil, and citronella oil and which is characterized by the fact that it remains thin and free-flowing under all conditions and does not gum.

2. A lubricating fluid for the purpose described, consisting of an emulsion containing water one gallon, soap (chip, flake or powder) one-fourth ounce, the soap being dissolved in the water, kerosene oil two gallons, and oil of citronella three ounces.

WILLIAM G. KLITZKE.

35

40